

# United States Patent Office

3,361,673

Patented Jan. 2, 1968

1

3,361,673

## LUBRICATING OIL COMPOSITIONS CONTAINING ALKENYL SUCCINIMIDES OF TETRAETHY- ENE PENTAMINE

Frank A. Stuart, Orinda, Robert G. Anderson, Novato, and Alan V. Drummond, Richmond, Calif., assignors to Chevron Research Company, a corporation of Delaware

No Drawing. Filed Aug. 24, 1959, Ser. No. 835,437  
6 Claims. (Cl. 252—51.5)

This invention pertains to lubricating oil compositions having incorporated therein metal-free detergents. These particular metal-free detergents are N-substituted polyamine alkenyl succinimides.

Alkenyl succinic anhydrides and numerous derivatives thereof are well known in the art. For example, alkenyl succinic anhydrides in which the alkenyl radical contains from 5 to 20 carbon atoms are taught as corrosion inhibitors in lubricating oil compositions. Also, products obtained by reacting such alkenyl succinic acid anhydrides with monoamines are taught as ferrous corrosion inhibitors for lubricating oil compositions.

However, the above known alkenyl succinimides are not useful as detergents in lubricating oil compositions. In contrast thereto, the N-substituted polyamine alkenyl succinimides which are described herein are new compounds which are useful as detergents in lubricating oil compositions.

Present day internal combustion engines operate at high speeds and high compression ratios. When used in the so-called city stop-and-go driving, which includes the greater part of the driving condition for a large percentage of today's automobiles, the internal combustion engines do not reach the most efficient operating temperature. Under city driving conditions, large amounts of partial oxidation products are formed, and reach the crankcase of the engine by blowing past the piston rings. Most of these partial oxidation products are oil insoluble, tending to form deposits on the various operating parts of the engine, such as the pistons, piston rings, etc. For the purpose of preventing the deposition of these products on the various engine parts, it is necessary to incorporate detergents in the lubricating oil compositions, thus keeping these polymeric products highly dispersed in a condition unfavorable for deposition on metals.

For the most part, the various detergents which are added to crankcase oils to reduce this formation of sludges and varnishes are metal organic compounds, particularly those compounds wherein the metal is linked to an organic group through an oxygen atom. Although these metal-containing organic compounds have some effectiveness as detergents for dispersing the precursors of deposits within the oil itself rather than permitting them to form added deposits on the engine parts, they have the disadvantage of forming ash deposits in the engine. These ash deposits lower engine performance by fouling plugs and valves, and contributing to preignition.

II



It is a particular object of this invention to provide

2

lubricating oil compositions which are compounded with a metal-free detergent.

Therefore, in accordance with this invention, it has been discovered that lubricating oil compositions particularly useful for heavy duty service are obtained by incorporating N-substituted monoalkenyl succinimides derived from tetraethylene pentamine in oils of lubricating viscosity.

By the use of lubricating oil compositions containing the N-substituted alkenyl succinimides described herein, diesel and gasoline engine parts remain remarkably free of deposits and varnish, even under severe operating conditions.

These new compounds, which are monoalkenyl succinimides of tetraethylene pentamine, have the formula:



wherein R is a hydrocarbon radical having a molecular weight from about 400 to about 3000; that is, R is a hydrocarbon radical containing about 30 to about 200 carbon atoms.

These alkenyl succinimides of tetraethylene pentamine can be prepared by reacting maleic anhydride with an olefinic hydrocarbon, followed by reacting the resulting alkenyl succinic anhydride with tetraethylene pentamine. The "R" radical of the above formula, that is, the alkenyl radical, is derived from an olefin containing from 2 to 5 carbon atoms. Thus, the alkenyl radical is obtained by polymerizing an olefin containing from 2 to 5 carbon atoms to form a hydrocarbon having a molecular weight ranging from about 400 to about 3000, more preferably, 900 to 1200. Such olefins are exemplified by ethylene, propylene, 1-butene, 2-butene, isobutene, and mixtures thereof. Since the methods of polymerizing the olefins to form polymers thereof is immaterial in the formation of the new compound described herein, any of the numerous processes available can be used therefor.

The preparation of N-substituted monoalkenyl succinimides derived from tetraethylene pentamine can be described generally by the following equations, using a polymer of isobutene as an example of the alkenyl radical:



wherein n has a value of about 7 to about 50.

The above reaction between a polyolefin and maleic anhydride is an uncatalyzed addition reaction which should not be confused with a copolymerization reaction such as that obtained with a vinyl monomer and maleic anhydride. While the general reaction of an olefin and maleic anhydride is well known for olefins of low molecular weight (e.g., olefins of 18 carbon atoms), no previous work has been done with maleic anhydride and the high molecular weight olefins as described herein.

The reaction set forth and described by Equation I hereinabove can proceed in a mol ratio of the polyolefin to the maleic anhydride of 1:1 to 1:10, preferably from 1:1 to 1:5. The reaction temperature can vary from 300° F. to 450° F. Because of the greater yield of products obtained thereby, it is preferred to use the high range of temperatures (e.g., 375° F. to 450° F.).

In the second step of the reaction as exemplified by Equation II hereinabove, the yield of the imide is extremely high even though the reactants are used in equal molar ratios. This is surprising, since under the conditions of the reaction there is an excess of secondary amino groups over primary amino groups, and any reaction with the secondary amino groups would lead to amide formation; thus, preventing imide formation.

The reaction described by Equation II hereinabove can be made at 220° F. to 500° F., preferably from 300° F. to 400° F. The alkenyl succinic anhydride and the tetraethylene pentamine are reacted in about equal molar quantities.

Since the reaction between the polyolefin and maleic anhydride may not go to completion, the resulting alkenyl succinic anhydride may contain some unreacted polyolefin. As it may not be desirable to separate out this unreacted polyolefin at this stage, the resulting imide formed by reaction of the alkenyl succinic anhydride and the diamine will contain this polyolefin as an impurity which can be a diluent in the formation of lubricating oil compositions. However, if it is so desired, this unreacted polyolefin can be removed by precipitation, for example, by acetone or methanol from a hydrocarbon solution.

Lubricating oils which can be used as base oils include a wide variety of lubricating oils, such as naphthenic base, paraffin base, and mixed base lubricating oils, other hydrocarbon lubricants, e.g., lubricating oils derived from coal products, and synthetic oils, e.g., alkylene polymers (such as polymers of propylene) butylene, etc., and the mixtures thereof, alkylene oxide-type polymers (e.g., propylene oxide polymers) and derivatives, including alkylene oxide polymers prepared by polymerizing the alkylene oxide in the presence of water or alcohols, e.g., ethyl alcohol, dicarboxylic acid esters (such as those which are prepared by esterifying such dicarboxylic acids as adipic acid, azelaic acid, suberic acid, sebacic acid, alkanol succinic acid, fumaric acid, maleic acid, etc., with alcohols such as butyl alcohol, hexyl alcohol, 2-ethyl hexyl alcohol, dodecyl alcohol, etc.), liquid esters of acids of phosphorus, alkyl benzenes (e.g., monoalkyl benzene such as dodecyl benzene, tetradecyl benzene, etc., and dialkyl benzenes (e.g., n-nonyl 2-ethyl hexyl benzene); polyphenyls (e.g., biphenyls and terphenyls), alkyl biphenyl ethers, polymers of silicon (e.g., tetraethyl silicate, tetra-isopropyl silicates, tetra(4-methyl-2-tetraethyl) silicate, hexyl (4-methyl-2-pentoxy) disiloxane, poly(methyl) siloxane, poly(methylphenyl) siloxane, etc. Synthetic oils of the alkylene oxide-type polymers which may be used include those exemplified by the alkylene oxide polymers.

The above base oils may be used individually or in combinations thereof, wherever miscible or wherever made so by the use of mutual solvents.

The alkenyl succinimides of tetraalkylene pentamine can be used in oils of lubricating viscosity in amounts of 0.1% to 80%, by weight, preferably 0.25% to 5%, by weight.

The preparation of the alkenyl succinimides of tetra-

alkylene pentamine is illustrated in the following examples.

*Example I.—Preparation of polybutenyl succinic anhydride*

A mixture of 1000 grams (1 mol) of polybutene having a molecular weight of about 1000 and 98 grams (1 mol) of maleic anhydride was heated at 410° F. in a nitrogen atmosphere with agitation for a period of 24 hours. The reaction mixture was cooled to 150° F. and 700 cc. of hexane added; after which the mixture was filtered under vacuum. After vacuum distillation to remove the hexane from the filtrate, the product was maintained at 350° F. at an absolute pressure of 10 mm. Hg for one hour to remove traces of maleic anhydride. The crude polybutenyl succinic anhydride thus prepared had a saponification number of 79.

*Example II.—Preparation of tetraethylenepentamine derivative of the polybutenyl succinic anhydride of Example I hereinabove*

A mixture of 84 grams (0.45 mol) of tetraethylene pentamine and 702 grams (0.45 mol) of the polybutenyl succinic anhydride of Example I hereinabove, was blended with agitation at 125° F. in a nitrogen atmosphere. The temperature was increased to 400° F. during a period of one hour, after which the absolute pressure was reduced to about 200 mm. Hg during a period of 30 minutes to facilitate the removal of water. The reaction mixture was then allowed to reach room temperature at this reduced pressure. The reaction product contained 5.1% nitrogen (theory=5.4%). Infra-red analysis showed that the reaction product was an imide containing a polybutene side chain.

As detergents for lubricating oil compositions, the compounds of this invention are more effective than alkenyl succinimides having fewer nitrogen atoms in the amine portion of the molecule, and succinimides having less than 30 carbon atoms in the alkenyl radical. The use of amyl amine, for example, in place of tetraethylene pentamine in the preparation of the succinimide, results in a product which is ineffective as a detergent in lubricating oil compositions.

Table I hereinbelow presents data obtained with lubricating oil compositions containing N-substituted monoalkenyl succinimides derived from tetraethylene pentamine.

The monoalkenyl succinimide used was an N-substituted succinimide derived from tetraethylene pentamine wherein in the alkenyl radical had a molecular weight of about 1000, which alkenyl radical was a polymer of isobutene.

The tests were made in a Caterpillar L-1 engine according to Supplement I conditions for a period of 120 hours as described in the Coordinating Research Council Handbook, January, 1946.

The "PD Nos." refer to the piston discoloration rating. After the engine test, the three piston lands are examined visually. To a piston skirt which is completely black is assigned a PD number of 800; to one which is completely clean, a PD number of 0; to those intermediate between completely black and completely clean are assigned PD numbers intermediate in proportion to the extent and degree of darkening.

The "G.D. Nos." refer to the percentage deposits in the piston ring grooves; and 0 evaluation being a clean groove; and a number of 100 being a groove full of deposits.

The base oils were California SAE 30 base oils.

The dithiophosphate was a zinc salt of a mixed dialkyl dithiophosphate wherein one of the alkyl radicals contained 4 carbon atoms and the other alkyl radical contained 5 carbon atoms. The dithiophosphate was present in the lubricating oil compositions in an amount of 18 millimols per kilogram (i.e., 18 mm./kg.) of finished product, based on the metal content.



wherein R is a hydrocarbon radical having a molecular weight of from about 900 to about 3000.

2. A lubricating oil composition consisting essentially of an oil of lubricating viscosity, and from about 0.1% to about 80%, by weight, of a monoalkenyl succinimide of tetraethylene pentamine of the formula:



wherein R is a hydrocarbon radical derived from a polymer of an olefin containing from 2 to 5 carbon atoms, said polymer having a molecular weight in the range of about 900 to about 3000.

3. A lubricating oil composition consisting essentially of an oil of lubricating viscosity, and from about 0.1% to about 80%, by weight, of a monoalkenyl succinimide of tetraethylene pentamine of the formula:



wherein R is a hydrocarbon radical derived from a polymer of an olefin containing from 2 to 5 carbon atoms, said polymer having a molecular weight in the range of about 900 to about 1200.

4. A lubricating oil composition comprising a major proportion of a petroleum lubricating oil, and from about 0.25% to about 5%, by weight, of an N-substituted monoalkenyl succinimide of the formula:



wherein R is a polymer of isobutene having a molecular weight of about 1000.

5. A lubricating oil composition comprising a major proportion of a petroleum lubricating oil, and from about 0.25% to about 5%, by weight, of an N-substituted monoalkenyl succinimide of the formula:

5



10

wherein R is a polymer of an olefin containing 4 carbon atoms, said polymer having a molecular weight of about 1000.

15 6. A lubricating oil composition comprising a major proportion of a mineral oil of lubricating viscosity and from about 0.1% to about 5% by weight of an imide prepared by reacting an alkenyl succinic anhydride having the structural formula

20



25

in which structural formula R is a substantially aliphatic hydrocarbon radical of from 50 to 200 carbon atoms, with an equal molar quantity of tetraethylene pentamine 30 at a temperature in the range of 220° F. to 360° F.

#### References Cited

#### UNITED STATES PATENTS

- |    |           |         |                    |           |
|----|-----------|---------|--------------------|-----------|
| 35 | 2,490,744 | 12/1949 | Trigg et al. ----- | 252—392 X |
|    | 2,604,451 | 7/1952  | Rocchini -----     | 252—51.5  |
|    | 2,638,450 | 5/1953  | White et al. ----- | 252—51.5  |

DANIEL E. WYMAN, Primary Examiner.

40 PATRICK P. GARVIN, JULIUS GREENWALD,  
Examiners.

G. O. ENOCKSON, Assistant Examiner.

UNITED STATES PATENT OFFICE  
CERTIFICATE OF CORRECTION

Patent No. 3,361,673

January 2, 1968

Frank A. Stuart et al.

It is certified that error appears in the above identified patent and that said Letters Patent are hereby corrected as shown below:

Column 1, line 57, "plugs" should read -- spark plugs --. Columns 1 and 2, formula II should appear as shown below:



Column 3, line 46, "(such as polymers of propylene)" should read -- (such as polymers of propylene, --. Column 4, line 6, "of polybutene" should read -- of a polybutene --. Column 6, line 35, "I" should read -- IV --; same column 6, lines 69 to 75, the formula should appear as shown below:



Signed and sealed this 16th day of December 1969.

(SEAL)

Attest:

EDWARD M. FLETCHER, JR.  
Attesting Officer

WILLIAM E. SCHUYLER, JR.  
Commissioner of Patents